

## UNITED STATES PATENT OFFICE

2,415,724

## CHROMIUM PLATING

Frank H. Beall, Maplewood, N. J.

No Drawing. Original application October 15, 1936, Serial No. 105,799. Divided and this application November 6, 1939, Serial No. 303,077

4 Claims. (Cl. 204—32)

1

The invention relates to the electrodeposition of chromium and is more particularly concerned with a process employing a novel chromium plating solution and special preparation of the metal surfaces preliminary to the plating operation per se.

This application is a division of my copending application Serial No. 105,799, filed October 15, 1936, now Patent No. 2,182,244, dated December 5, 1939.

The object of the invention is to provide a process of chromium plating which is an improvement on present practices particularly in being less sensitive to variations in the factors involved in chromium plating and in the quality of the chromium plate produced.

A common practice in chromium plating is to use a plating bath composed essentially of a water solution of chromic acid ( $\text{CrO}_3$ ) and a sulphate or sulphuric acid, the content of chromic acid varying, in general, from 150 to 450 grams per liter and the sulphate, estimated as  $\text{SO}_4$ , being preferably about 1% of the  $\text{CrO}_3$  content. The extreme theoretical range for the ratio of  $\text{SO}_4$  to  $\text{CrO}_3$  is from 1 to 50 to 1 to 250, i. e. the  $\text{SO}_4$  amounts to from 2% to 0.4% of the  $\text{CrO}_3$  content. But in actual practice the ratio of  $\text{SO}_4$  to  $\text{CrO}_3$  is between 0.66% and 1.15%. Seemingly slight departures from the prescribed conditions of the  $\text{SO}_4$  to  $\text{CrO}_3$  ratio, the concentration of the  $\text{CrO}_3$ , and the temperature result in defective plating.

In contrast with the generally accepted practice, I have found that by the use of other metals than chromium and of their soluble salts of chromic acid, particularly bichromates, a chromium plating process is produced of lower sulphate content which has the desired advantages over known methods. In the following description I will refer specifically to salts of sodium, such salts being more readily available commercially, but it should be understood that it is not intended to confine the invention to the use of sodium salts, as soluble salts of potassium, ammonium, zinc, and other bases are suitable. The essential characteristic of the additional metal is that it forms with the chromic acid a soluble bichromate, the metal of which does not deposit or the salt precipitate or form a colloidal solution. Bichromates of limited solubility can be mixed with those of greater solubility.

There are several ways in which the plating bath can be made up. A preferred method, disclosed in my prior application, Serial No. 686,069, filed August 21, 1933, of which the parent application Serial No. 105,799, above referred to, is in

2

part a continuation, comprises mixing the following:

|                                               |   |        |     |
|-----------------------------------------------|---|--------|-----|
| Chromic acid ( $\text{CrO}_3$ )               | — | pounds | 100 |
| Sodium carbonate ( $\text{Na}_2\text{CO}_3$ ) | — | do     | 36½ |
| Alumina hydrate (commercial)                  | — | ounces | 19  |
| Water                                         | — | pounds | 8   |

The chromic acid and alumina hydrate are mixed first and then the sodium carbonate and water added in alternating increments, the final product being about 125 lbs. of a yellowish powder. (The final content of  $\text{SO}_4$  in this mixture as shown by analyses is about .21-.22% of the powder or about .27% of the total  $\text{CrO}_3$ .) The plating bath is made up by dissolving the mixture in water, about three pounds to the gallon being preferred.

The composition may be obtained by direct admixture of  $\text{CrO}_3$  and sodium bichromate or equivalent chromate, the choice of reagents to convert the  $\text{CrO}_3$  into bichromates or to supply the chromate or bichromate being merely a question of relative cost of materials of the necessary purity.

The "alumina hydrate" employed is a commercial product containing a fairly definite proportion, about 12% of  $\text{SO}_3$ . The alumina hydrate, being a bulky material, facilitates uniform mixing. The commercial  $\text{CrO}_3$  also contains sulphate as an impurity as may also the  $\text{Na}_2\text{CO}_3$ . But in the actual practice of my invention, the total sulphate is preferably around or below 0.1 oz. per gallon of bath as compared with three or four times as much in the conventional high acid bath. The above mixture will give about 0.1 oz. per gallon of plating solution containing 3 lbs. of the mixture. Of course, other sulphate carriers than the alumina hydrate can be used, such as sodium sulphate in proper proportions, the essential ingredients being free  $\text{CrO}_3$ , the salt of  $\text{CrO}_3$  and the catalytic acid radical preferably  $\text{SO}_4$ .

The exact proportion of the hexavalent chromium present in the form of the salt (considering the salt to be bichromate) is not critical, 70% being generally sufficient. Solutions in which 80% is in the combined form have a slightly higher throwing power but lower conductivity. Much above 80% results in difficulties in obtaining a good plate. Operating conditions will therefore affect the ratio selected, for example, the relative desirability of lower resistance and of higher throwing power. In general, 70% is recommended and less than 60% is not preferred. The preferred method outlined above gives neutralization of chromic acid to bichromate of approximately 70%.

Variations in concentration of the bath content are also possible. These variations are limited on the upper side by solubility of the compound and on the lower side by a darkening or lack of uniformity of the deposit. I have, therefore, found it desirable to maintain the mixture at not less than 30 oz. per gallon. The concentration of free  $\text{CrO}_3$ , however, should be maintained at not less than 5 oz. per gallon even when lower concentrations of total chromium are used.

I have found that variations in the sulphate concentration in this plating solution over a very wide range when operated as hereinafter described give results that produce a flat bright plate characteristic curve. This curve from a 15 concentration of about .25 ounce of  $\text{SO}_4$  per gallon on down to the lower limit practically possible by operating with commercial  $\text{CrO}_3$  shows a substantially uniform bright plate range. The range, however, is somewhat wider at the lower 20  $\text{SO}_4$  concentrations. It was for this reason and also for a minimum etching action of the solution that I prefer the .1 oz.  $\text{SO}_4$  per gallon concentration, which concentration can be conveniently maintained with average commercial  $\text{CrO}_3$  even when taking into account the consumption factor which tends to build up  $\text{SO}_4$  from this impurity in the  $\text{CrO}_3$  consumed. With much above the .25 oz.  $\text{SO}_4$  per gallon, however, the bright plate range 25 rapidly narrows, as reduced chromium oxides are formed at a faster rate than they are dissolved by the solution. This difficulty is of course greater at lower mixture concentrations, which is the reason for choosing the approximately 48 oz. per gallon solution concentration as the preferred one. While higher solution concentrations possess certain advantages, the drag out factor also increases, causing increased cost.

I have found that, by varying the proportions of chromic acid salts, the ratio of hexavalent chromium to  $\text{SO}_4$  can be widely varied and plating solutions obtained which are very low in  $\text{SO}_4$  content. For example, a solution of a high grade of chromic acid containing 0.085%  $\text{SO}_4$ , which without addition of more sulphate will give no indication of plating at normal current densities, can be made to plate upon neutralizing a substantial part of the chromic acid with sulphate-free  $\text{NaOH}$ . In such solution the ratio of hexavalent chromium to  $\text{SO}_4$  is about 1180 to 1.

Good results with such solution have been obtained when the  $\text{CrO}_3$  was neutralized to about 80% (estimating the neutralized  $\text{CrO}_3$  to be in the form of sodium bichromate) leaving 20% of the  $\text{CrO}_3$  as free acid, with the total original  $\text{CrO}_3$  content about 40 oz. to the gallon. Consistent plating has been obtained with the neutralization from 75% to 85% but if as much as 90% of the  $\text{CrO}_3$  is neutralized no plating at all is obtained. It will be noted that, with 75% neutralization, the  $\text{SO}_4$  is 0.34% of the free or unneutralized  $\text{CrO}_3$ , and at 90% neutralization the  $\text{SO}_4$  is 0.85% of the free  $\text{CrO}_3$ .

It is my belief that the salts thus introduced serve to dissolve or to maintain in solution the salts or oxides of reduced chromium which otherwise deposit along with metallic chromium and cause iridescence, splotches, or dark deposits. The bath differs, however, from all former chromium plating baths, of which I am aware, in the following particulars: first, the total sulphate radical relative to the total  $\text{CrO}_3$  radical present is lower than is practicable in any known commercial bath. (This feature lowers the acidity and reduces the oxidizing and etching effect on

the metal surfaces to be plated); second, the sulphate radical present has no definite relation either to the neutralized  $\text{CrO}_3$  present or to the unneutralized radical present.

The maintenance of the solution is very simple. The proportions are much less critical than in the high acid baths in present use and commercial baths have been controlled over long periods by tests of the Baumé gravity only, by merely adding material of the original composition plus a percentage of  $\text{CrO}_3$  to compensate for the consumption of the  $\text{CrO}_3$ . Frequent chemical analyses are unnecessary.

In plating with my low acid bath it has been found that the deposits are whiter, i. e., they are free from the bluish cast of conventional chromium plate. Also the deposit is less brittle and there is a practically complete absence of fine cracks commonly experienced with higher acid ratios.

The characteristics of my bath of low acid content not only enable it to plate chromium directly upon articles, such as zinc-base die castings, or articles of lead, pewter or silver, that cannot be satisfactorily plated in the usual bath, but also enables it to plate successfully on nickel, copper, brass etc. after the work has been subjected to preliminary cleaning and etching operations which are adapted to the particular metal surface to be plated.

The bright plate range is not controlled by the chemical composition of the solution and temperature alone, but is very largely dependent at 35 the lower  $\text{SO}_4$  concentrations on the preliminary treatment of the metal surface.

The invention accordingly contemplates the use of certain preliminary treatments adapted to and in combination with the subsequent plating 40 in my low acid bath. By these treatments I apparently invisibly etch or roughen the metal surfaces so that the proper bond is produced in my plating solution to which the work is subsequently subjected.

In determining the ingredients of the etch 45 solution, the products of their reaction should be soluble in the etch solution itself.

For nickel I use a mixture of an oxidizing reagent such as  $\text{CrO}_3$  and an acid such as  $\text{HCl}$ . A properly etched surface, free from insoluble oxidation products, is obtained for the above preferred plating bath by the following solution:

|                         | Ounces per gallon |
|-------------------------|-------------------|
| 55 $\text{CrO}_3$ ----- | 2                 |
| NaCl -----              | .04 to .06        |

The concentration of the chlorine radical is the determining factor; and the  $\text{CrO}_3$  has to be made sufficiently concentrated to act as a dilute 60 acid wash to neutralize any alkali which may carry over from the usual previous cleaning operation.

An etch solution involving an increased amount 65 of acid radical and a bichromate, such as sodium or ammonium bichromate, results in a wider plating range for the truly bright plate. For example, such an etch solution may be as follows:

|                               | Ounces per gallon |
|-------------------------------|-------------------|
| 70 Sodium bichromate-----     | 20                |
| $\text{CrO}_3$ -----          | 2                 |
| NaCl -----                    | .04               |
| $\text{H}_2\text{SO}_4$ ----- | .1                |

The .1 of an ounce of  $\text{H}_2\text{SO}_4$  is substantially 75 .5% of the 20 oz. of the sodium bichromate used.

This is the normal sulphate impurity in commercial sodium bichromate.

Instead of adding sodium bichromate, equivalent amounts of soda ash and chromic acid may be added. As commercial soda ash contains sodium chloride as an impurity, the employment of this combination would operate to add additional sodium chloride.

The procedure for the plating of a nickel surface is:

(a) Clean work in cleaning solution and rinse with water.

(b) Etch for about ten seconds in nickel etch solution at room temperature. Time is not critical. Then rinse in water.

(c) Enter work in the chromium tank, making sure that it is well wet with the plating solution before making contact with the cathode bar.

The plating solution of my invention possesses a good bright plate range on nickel, even at temperatures of 110° F. but the best general range on this metal is 80-90° F.

While I have outlined different etching solutions which I have found preferable for my preferred plating solution, I must make clear that these exact proportions for the etching solutions will not be the optimum for the entire range of variation in plating solutions having sulphate radical concentrations below approximately .65 percent, but would have to be varied according to the departures from the preferred plating solutions and directions given above. It should be understood that it is not intended to confine the invention to the use of the preferred nickel etching solution described above. Since I have found that the salts of both hydrochloric and sulphuric acid react as acids through ionization in the presence of weak acids, such as chromic acid, it is obvious that hydrochloric or sulphuric or other strong acids such as hydrofluoric acid can be used in combination with an oxidizing reagent, such as chromic acid to make suitable nickel etching solutions. In the substitution of other strong acids for hydrochloric acid, it should be observed that the most suitable proportions of acid will not depend upon the comparison with hydrochloric acid upon the basis of hydrogen ion concentration. Different acids have different etching characteristics in the presence of an oxidizing reagent, such as chromic acid. The proper proportions for other strong acids will easily be found. When the action of the etching bath is too strong, un-plated areas form on the work in the plating operation; when too weak, the throwing power is poor and the resulting plate hazy.

The etching action of the preferred plating solution on nickel is practically negligible; but if higher ratios of SO<sub>4</sub> to total CrO<sub>3</sub> are used, the etching action is not negligible and must be taken into account and allowed for in determining the degree of etching action desired in the preliminary etching operation.

While I have described the use of plating baths containing bichromate and low in SO<sub>4</sub> concentration with my etching baths, it should be understood that the invention is not to be confined to the use of my etching baths with such plating solutions, for my etching baths can be usefully employed with plating solutions containing little or no bichromate (representing neutralizations of CrO<sub>3</sub> from 60 per cent down to zero per cent) but containing SO<sub>4</sub> in lower concentrations than .65 per cent. Although such plating solutions have a greater etching action than similar baths containing substantial amounts of bichromate as

described above, they are still useful for plating with my etching solutions. If the SO<sub>4</sub> concentration of such baths is reduced, the etching action is correspondingly reduced until it practically ceases at the lowest concentrations. Higher SO<sub>4</sub> concentrations though still below .65 per cent result in an etching action which must be taken into account and allowed for in determining the degree of etching action desired in the preliminary etching operation. This etching action of the higher SO<sub>4</sub> concentrations (though still below .65 per cent) is little affected by small amounts of bichromate. But if the proportion of bichromate is increased, the effect is to diminish the etching action until at the preferred percentages of neutralization, the etching action is reduced to minimum proportions.

The advantages of my process claimed herein over the present high-acid method are as follows:

(1) On nickel the ease with which a true bright plate may be obtained even with irregular hand operation in the plating bath.

(2) No changes take place in the etching solution to upset the equilibrium so that control is greatly simplified.

(3) The plating solution is much less sensitive to the proportions of the chemical components present, e. g., Na, CrO<sub>3</sub>, and SO<sub>4</sub>, so that its maintenance is much less critical. There is no necessity to maintain a substantially constant ratio of SO<sub>4</sub> to either the total CrO<sub>3</sub> present or to the free CrO<sub>3</sub> present.

(4) The temperature may vary over a considerable range without affecting the results.

While I have referred above to the sulphate content, it should be understood that the invention is not limited to such acid radical additional agent or "catalyst." Other such addition agents known in the art, fluorides, fluosilicates, etc. may be employed in reduced amounts in accordance with the present invention. The impurity present in the CrO<sub>3</sub> and other materials, however, must be taken into account and corresponding reduction made in the additions of such catalysts. As sulphate is already present in the commercial raw material in amounts that roughly correspond with that used, the use of such equivalent known "catalysts" would largely depend on obtaining a raw material of greater purity than presently commercially available.

I claim:

1. The process of preparing the surface of nickel for electrodeposition of chromium thereon comprising subjecting the surface to the non-electrolytic action of a solution containing chromic acid, bichromate, sulphate and sodium chloride, said solution being composed substantially as follows: 20 oz. per gallon sodium bichromate, 2 oz. per gallon CrO<sub>3</sub>, .04 oz. per gallon NaCl, and .1 oz. per gallon H<sub>2</sub>SO<sub>4</sub>.

2. The process of plating chromium on a surface composed essentially of nickel which comprises; first subjecting the surface to the non-electrolytic action of a solution containing chromic acid as an oxidizing agent and the acid radical of a strong acid to prepare the said metal surface for plating chromium thereon; washing said prepared surface; thereafter immersing the same in a plating bath containing an aqueous solution of chromic acid in part free and in part combined as an alkali salt of chromic acid, the total chromic acid being at least about 30 oz. per gallon of solution and the free acid constituting approximately 20 to 40% of the total, and sulphate catalyst to the amount of not over ap-

proximately .65% of the total chromic acid; and supplying plating current to said surface.

3. The process of plating chromium upon a surface composed largely or entirely of nickel which includes; subjecting the surface to the non-electrolytic action of a solution containing chromic acid as an oxidizing agent and the acid radical of a strong acid such as hydrochloric acid, sulphuric acid and hydrofluoric acid to prepare the said metal surface for plating chromium thereon; washing said prepared surface; thereafter immersing said surface in a plating bath containing an aqueous solution of chromic acid in part free and in part combined as a metal salt of chromic acid, the metal of which does not deposit or the salt precipitate to form a colloidal solution, the total chromic acid being at least about 30 oz. per gallon of solution and the free acid constituting approximately 20 to 40% of the total, and a catalyst consisting of at least one of the following class of catalysts, sulphates, fluorides, and fluosilicates to the amount of not over approximately .65% of the total chromic acid; and supplying plating current to said surface.

4. The process of plating chromium upon a metal surface composed largely or entirely of nickel which includes; treating the metal surface in a solution containing about 20 oz. per gallon sodium bichromate, about 2 oz. per gallon  $\text{CrO}_3$ , about .04 oz. per gallon  $\text{NaCl}$ , and about .1 oz. per gallon  $\text{H}_2\text{SO}_4$ ; washing said treated surface;

thereafter immersing the surface in a plating bath comprising an aqueous solution containing free chromic acid, a soluble bichromate, and a sulphate catalyst, the total chromic acid being about 30 to 50 oz. per gallon of solution, the free chromic acid being about 30% of the total chromic acid and the sulphate catalyst being approximately .1 oz. per gallon; and supplying plating current to said surface.

10

15

20

25

30

FRANK H. BEALL

## REFERENCES CITED

The following references are of record in the file of this patent:

## UNITED STATES PATENTS

| Number    | Name                | Date          |
|-----------|---------------------|---------------|
| 2,127,640 | Brown et al. -----  | Aug. 23, 1938 |
| 1,985,308 | Bornhauser -----    | Dec. 25, 1934 |
| 1,917,188 | Eaton -----         | July 4, 1933  |
| 1,903,130 | Phillips -----      | Mar. 28, 1933 |
| 1,787,477 | Hanley et al. ----- | Jan. 6, 1931  |

## FOREIGN PATENTS

| Number  | Country       | Date         |
|---------|---------------|--------------|
| 474,559 | British ----- | Nov. 3, 1937 |

## OTHER REFERENCES

Prin. of Electro Plating & Electro Forming, Blum & Hogaboom, 2nd ed. (1930), pub. by McGraw-Hill Bk. Co., N. Y., pp. 293, 306. (Copy in Div. 56.)